# EUROPEAN PATENT SPECIFICATION

(11) **EP 0 664 843 B1**
(45) Date of publication and mention of the grant of the patent: **29.10.1997**
(21) Application number: 93921473.0
(22) Date of filing: 09.09.1993
(51) Int. Cl.: D21F 3/08, D21G 1/02

(54) **A METHOD OF MANUFACTURING A COVER FOR A PRESS ROLL**
VERFAHREN ZUR HERSTELLUNG EINER PRESSWALZENBEKLEIDUNG
PROCEDE DE FABRICATION D'UNE ENVELOPPE POUR UN ROULEAU EXPRIMEUR

(30) Priority: 16.10.1992 US 962636
(43) Date of publication of application: 02.08.1995
(73) Proprietor: BELOIT TECHNOLOGIES, INC., Wilmington, DE 19801-1622 (US)
(72) Inventor: BONANDER, James, Clarks Summit, PA 18411 (US); SLAGOWSKI, Eugene, L., Waverly, PA 18471 (US)
(74) Representative: Schmitz, Jean-Marie
(86) International application number: US9308537
(87) International publication number: WO9409208

(56) References cited:
- EP-A- 0 146 342
- EP-A- 0 487 477
- DE-A- 2 330 565
- GB-A- 2 057 092
- US-A- 3 069 304

## Description

### Background of the Invention

### Field of the Invention

The present invention relates to a method of manufacturing a cover for a press roll. More specifically, the present invention relates to a method of manufacturing a cover for a press roll which includes spirally winding reinforcing material around the press roll.

### Information Disclosure Statement

In the papermaking art, a formed web is guided through a press section for removing water from the web.

Steel press rolls have been covered with rubber or synthetic material in order to enhance the water removing capability of the press.

Often, it has been the practice to add filler particles to the rubber compounds prior to application of the rubber compound to the steel roll shell in order to change the hardness of the resultant cover.

Additionally, fillers have been added to urethane in order to increase the hardness of the cover.

However, more recently, it has been found advantageous to impregnate reinforcing material with a urethane material and to spirally wind the same onto a roll shell. However, such spiral winding of the reinforcing material does not readily permit the addition thereto of the aforementioned filler particles.

The present invention overcomes the problem of adding filler to the spirally wound reinforcing material by applying the filler to an epoxy matrix prior to the application of the mixture to the reinforcing material.

Therefore, the present invention provides a method of manufacturing a cover for a press roll that overcomes the aforementioned inadequacies of the prior art arrangements and which makes a considerable contribution to the art of manufacturing a cover for a press roll.

Other objects and advantages of the present invention will be readily apparent to those skilled in the art by a consideration of the detailed description contained hereinafter, taken in conjunction with the annexed drawings.

### Summary of the Invention

The present invention relates to a method of manufacturing a cover for a press roll. The method includes the steps of feeding an epoxy matrix into a container and agitating the matrix. Filler material is added to the matrix while the matrix is being agitated, and the matrix and filler are then conveyed to an application zone. Reinforcing material is unwound from a roll such that the material extends past the application zone. The agitated matrix and filler are applied to the unwound material during passage of the material past the application zone. The reinforcing material, together with the matrix and filler, are then spirally wound around the press roll such that the press roll is covered with the reinforcing material impregnated with the matrix and filler. The arrangement is such that the surface characteristics of the resultant cover are dependent on the amount and type of filler material added to the matrix.

In a more specific embodiment of the present invention, the epoxy matrix is a polymeric thermo-plastic matrix.

In another embodiment of the present invention, the matrix is a polymeric thermo-set matrix.

The filler material is composed of either mineral particles, synthetic particles or refractory particles.

The particles in one embodiment of the invention have a diameter less than one (1) millimeter, and in another embodiment of the present invention, the particles have a diameter of at least one (1) millimeter.

In another embodiment of the present invention, the filler material includes PTFE powder, together with glass fibers. In yet another embodiment of the present invention, the filler material includes PTFE powder, together with ceramic fibers.

Additionally, in another embodiment of the present invention, the filler material includes PTFE powder, together with quartz fibers and feldspar particles.

The reinforcing material is either a woven material, a knitted material, a braided material or a non-woven material.

The step of spirally winding the reinforcing material is carried out during the cross-linking of the matrix.

Many variations and modifications of the combination of method steps according to the present invention will be readily apparent to those skilled in the art by a consideration of the detailed description contained hereinafter.

### Brief Description of the Drawings

Figure 1 is a schematic view representing the step of feeding the epoxy matrix into a container and agitating the same;
Figure 2 is a similar view to that shown in Figure 1, but shows filler material being added to the matrix while the matrix is being agitated;
Figure 3 is a similar view to that shown in Figure 2, but shows the agitated matrix and filler being conveyed to an application zone and being applied to reinforcing material being unwound from a roll of reinforcing material; and
Figure 4 is a perspective view showing a press roll being spirally wound with the reinforcing material and matrix and filler according to the present invention.

### Detailed Description of the Drawings

Figure 1 is a schematic view illustrating a method of manufacturing a cover for a press roll shell according to the present invention. Figure 1 shows an epoxy matrix **10** disposed within a container **12**. The epoxy matrix **10** is being agitated by an agitator **14**.

Figure 2 is a similar view to that shown in Figure 1, but shows filler material **16** being added to the matrix **10** while the matrix **10** is being agitated within the container **12**.

Figure 3 is a similar view to that shown in Figure 2, but shows the agitated matrix **10** and filler **16** being conveyed and pumped via pump P to an application zone, generally designated **18**.

A roll **20** of reinforcing material **22** is unwound, as indicated by the arrow **26**, such that the reinforcing material **22** extends past the application zone **18**.

The agitated matrix and filler **10** and **16** are applied, as indicated by the arrow **26**, to the unwound material **22** during passage of the unwound material **22** past the application zone **18**.

Figure 4 is a perspective view of a press roll **28** and shows the roll **28** being spirally wound with the reinforcing material **22**, the matrix **10** and filler **16** having been previously applied to the reinforcing material **22**. The arrangement is such that the press roll **28** is covered with the reinforcing material **22**, which is impregnated with the matrix **10** and filler **16**. The surface characteristics of the resultant cover are consequently dependent on the amount and type of filler material **16** added to the matrix.

In specific embodiments of the present invention, the matrix **10** is either a polymeric thermo-plastic matrix or a polymeric thermo-set matrix.

The filler material **16** is either composed of mineral particles, synthetic particles or refractory particles.

In one embodiment of the present invention, the filler material **16** includes particles having a diameter of less than one (1) millimeter, and in another embodiment of the present invention, the filler material **16** includes particles having a diameter of at least one (1) millimeter.

Additionally, the filler material **16** includes either PTFE powder together with glass fibers, PTFE powder together with ceramic fibers, or PTFE powder together with quartz fibers and feldspar particles.

The reinforcing material **22** is either a woven material, a knitted material, a braided material or a non-woven material.

The step of spirally winding the reinforcing material **22** is carried out during the cross-linking of the matrix.

The present invention provides a method of manufacturing a roll cover which exhibits the required durometer hardness for the particular type of paper being pressed.

Such hardness of the cover is not only a requirement according to the type of paper being manufactured, but also a requirement according to the type of coating that will be applied thereto for subsequent calendering.

Additionally, roll covers of varying durometer hardness will be required dependent upon the type of furnish being used.

Although the present invention has been described with particular application to the provision of a cover for a press roll, it will be appreciated by those skilled in the art that such roll covers will also be applicable in soft calendering and the like.

## Claims

1. A method of manufacturing a cover for a press roll (28), said method comprising the steps of:
feeding an epoxy matrix (10) into a container (12);
agitating the epoxy matrix (10);
adding filler material (16) to the matrix (10) while the matrix is being agitated; and
spirally winding reinforcing material (22) with the matrix (10) and filler (16) applied thereto around the press roll (28) such that the press roll (28) is covered with the reinforcing material (22) impregnated with the matrix (10) and filler (16), the arrangement being such that the surface characteristics of the resultant cover are dependent on the amount and type of filler material added to the matrix (10),
characterized by the steps of:
conveying the agitated matrix (10) and filler (16) to an application zone (18);
unwinding a roll (20) of the reinforcing material (22) such that the unwound reinforcing material (22) extends through the application zone (18); and
applying the agitating matrix (10) and filler (16) to the unwound material (22) during passage of the unwound material past the application zone (18).

2. A method of manufacturing a cover as set forth in claim 1, characterized in that the feeding step includes:
feeding a polymeric thermo-plastic matrix (10) into the container (12).

3. A method of manufacturing a cover as set forth in claim 1, characterized in that the feeding step includes:
feeding a polymeric thermo-set matrix (10) in the container (12).

4. A method of manufacturing a cover as set forth in claim 1, characterized in that the step of adding filler material (16) includes:
adding mineral particles to the matrix (10).

5. A method of manufacturing a cover as set forth in claim 1, characterized in that the step of adding filler material (16) includes:
adding synthetic particles to the matrix (10).

6. A method of manufacturing a over as set forth in claim 1, characterized in that the step of adding filler material (16) includes:
adding refractory particles to the matrix (10).

7. A method of manufacturing cover as set forth in claim 1, characterized in that the step of adding filler material (16) includes:
adding material having a particle size less than one (1) millimeter in diameter.

8. A method of manufacturing cover as set forth in claim 1, characterized in that the step of adding filler material (16) includes:
adding material having a particle size of at least one (1) millimeter in diameter.

9. A method of manufacturing a cover as set forth in claim 1, characterized in that the step of adding filler material (16) includes:
adding PTFE powder, together with glass fibers.

10. A method of manufacturing a cover as set forth in claim 1, characterized in that the step of adding filler material (16) includes:
adding PTFE powder, together with ceramic fibers.

11. A method of manufacturing a cover as set forth in claim 1, characterized in that the step of adding filler material (16) includes:
adding PTFE powder, together with quartz fibers, together with feldspar particles.

12. A method of manufacturing a cover as set forth in claim 1, characterized in that the reinforcing material (22) is a woven material.

13. A method of manufacturing a cover as set forth in claim 1, characterized in that the reinforcing material (22) is a knitted material.

14. A method of manufacturing a cover as set forth in claim 1, characterized in that the reinforcing material (22) is a braided material.

15. A method of manufacturing a cover as set forth in claim 1, characterized in that the reinforcing material (22) is a non-woven material.

16. A method of manufacturing a cover as set forth in claim 1, characterized in that the step of spirally winding the reinforcing material (22) is carried out during the cross-linking of the matrix (10).

## Patentansprüche

1. Verfahren zum Herstellen einer Umhüllung für eine Preßwalze (28), wobei das Verfahren die Schritte beinhaltet:
Einbringen einer Epoxymatrix (10) in einen Behälter (12);
Umrühren der Epoxymatrix (10);
Zusetzen von Füllmaterial (16) zu der Matrix (10), während die Matrix umgerührt wird; und
spiralförmiges Wickeln von Verstärkungsmaterial (22), auf das die Matrix (10) und der Füllstoff (16) aufgetragen worden sind, um die Preßwalze (28) derart, daß die Preßwalze (28) mit dem mit der Matrix (10) und dem Füllstoff (16) getränkten Verstärkungsmaterial (22) umhüllt wird, wobei die Anordnung so getroffen wird, daß die Oberflächeneigenschaften der sich ergebenden Umhüllung von der Menge und dem Typ des Füllmaterials, das der Matrix (10) zugesetzt wird, abhängig sind,
gekennzeichnet durch die Schritte:
Fördern der umgerührten Matrix (10) und des Füllstoffes (16) zu einer Auftragszone (18);
Abwickeln einer Rolle (20) des Verstärkungsmaterials (22) derart, daß sich das abgewickelte Verstärkungsmaterial (22) durch die Auftragszone (18) erstreckt; und
Auftragen der umgerührten Matrix (10) mit dem Füllstoff (16) auf das abgewickelte Material (22) während des Vorbeigangs des abgewickelten Materials an der Auftragszone (18).

2. Verfahren zum Herstellen einer Umhüllung nach Anspruch 1, dadurch gekennzeichnet, daß der Schritt des Einbringens beinhaltet:
Einbringen einer polymeren thermoplastischen Matrix (10) in den Behälter (12).

3. Verfahren zum Herstellen einer Umhüllung nach Anspruch 1, dadurch gekennzeichnet, daß der Schritt des Einbringens beinhaltet:
Einbringen einer polymeren duroplastischen Matrix (10) in den Behälter (12).

4. Verfahren zum Herstellen einer Umhüllung nach Anspruch 1, dadurch gekennzeichnet, daß der Schritt des Zusetzens von Füllmaterial (16) beinhaltet:
Zusetzen von mineralischen Partikeln zu der Matrix (10).

5. Verfahren zum Herstellen einer Umhüllung nach Anspruch 1, dadurch gekennzeichnet, daß der Schritt des Zusetzens von Füllmaterial (16) beinhaltet:
Zusetzen von synthetischen Partikeln zu der Matrix (10).

6. Verfahren zum Herstellen einer Umhüllung nach Anspruch 1, dadurch gekennzeichnet, daß der Schritt des Zusetzens von Füllmaterial (16) beinhaltet:
Zusetzen von feuerfesten Partikeln zu der Matrix (10).

7. Verfahren zum Herstellen einer Umhüllung nach Anspruch 1, dadurch gekennzeichnet, daß der Schritt des Zusetzens von Füllmaterial (16) beinhaltet:
Zusetzen von Material, das eine Partikelgröße hat, die weniger als einen (1) Millimeter im Durchmesser beträgt.

8. Verfahren zum Herstellen einer Umhüllung nach Anspruch 1, dadurch gekennzeichnet, daß der Schritt des Zusetzens von Füllmaterial (16) beinhaltet:
Zusetzen von Material, das eine Partikelgröße hat, die wenigstens einen (1) Millimeter im Durchmesser beträgt.

9. Verfahren zum Herstellen einer Umhüllung nach Anspruch 1, dadurch gekennzeichnet, daß der Schritt des Zusetzens von Füllmaterial (16) beinhaltet:
Zusetzen von PTFE-Pulver zusammen mit Glasfasern.

10. Verfahren zum Herstellen einer Umhüllung nach Anspruch 1, dadurch gekennzeichnet, daß der Schritt des Zusetzens von Füllmaterial (16) beinhaltet:
Zusetzen von PTFE-Pulver zusammen mit keramischen Fasern.

11. Verfahren zum Herstellen einer Umhüllung nach Anspruch 1, dadurch gekennzeichnet, daß der Schritt des Zusetzens von Füllmaterial (16) beinhaltet:
Zusetzen von PTFE-Pulver zusammen mit Quarzfasern, zusammen mit Feldspatpartikeln.

12. Verfahren zum Herstellen einer Umhüllung nach Anspruch 1, dadurch gekennzeichnet, daß das Verstärkungsmaterial (22) ein gewebtes Material ist.

13. Verfahren zum Herstellen einer Umhüllung nach Anspruch 1, dadurch gekennzeichnet, daß das Verstärkungsmaterial (22) ein gestricktes Material ist.

14. Verfahren zum Herstellen einer Umhüllung nach Anspruch 1, dadurch gekennzeichnet, daß das Verstärkungsmaterial (22) ein geflochtenes Material ist.

15. Verfahren zum Herstellen einer Umhüllung nach Anspruch 1, dadurch gekennzeichnet, daß das Verstärkungsmaterial (22) ein ungewebtes Material ist.

16. Verfahren zum Herstellen einer Umhüllung nach Anspruch 1, dadurch gekennzeichnet, daß der Schritt des spiralförmigen Wickelns des Verstärkungsmaterials (22) während der Vernetzung der Matrix (10) ausgeführt wird.

## Revendications

1. Procédé de fabrication d'un recouvrement pour un cylindre de presse (28), ledit procédé comprenant les étapes consistant à:
alimenter une matrice époxy (10) dans un récipient (12);
agiter la matrice époxy (10);
ajouter une matière de charge (16) à la matrice (10) tout en agitant la matrice (10); et
enrouler en spirale une matière de renforcement (22) sur laquelle on a appliqué la matrice (10) et la matière de charge (16) autour du cylindre de presse (28) de telle sorte que le cylindre de presse (28) est recouvert avec la matière de renforcement (22) imprégnée avec la matrice (10) et avec la matière de charge (16), l'arrangement étant tel que les caractéristiques superficielles du recouvrement résultant dépendent de la quantité et du type de la matière de charge ajoutée à la matrice (10);
caractérisé par les étapes consistant à:
acheminer la matrice agitée (10) et la matière de charge (16) à une zone d'application (18);
dérouler un rouleau (20) de la matière de renforcement (22) de telle sorte que la matière de renforcement déroulée (22) s'étend à travers la zone d'application (18); et
appliquer la matrice agitée (10) et la matière de charge (16) sur la matière déroulée (22) au cours du passage de la matière déroulée devant la zone d'application (18)

2. Procédé de fabrication d'un recouvrement selon la revendication 1, caractérisé en ce que l'étape d'alimentation englobe:
le fait d'alimenter une matrice thermoplastique polymère (10) dans le récipient (12).

3. Procédé de fabrication d'un recouvrement selon la revendication 1, caractérisé en ce que l'étape d'alimentation englobe:
le fait d'alimenter une matrice polymère thermodurcissable (10) dans le récipient (12).

4. Procédé de fabrication d'un recouvrement selon la revendication 1, caractérisé en ce que l'étape d'addition de la matière de charge (16) englobe:
le fait d'ajouter des particules minérales à la matrice (10).

5. Procédé de fabrication d'un recouvrement selon la revendication 1, caractérisé en ce que l'étape d'addition de la matière de charge (16) englobe:
le fait d'ajouter des particules synthétiques à la matrice (10).

6. Procédé de fabrication d'un recouvrement selon la revendication 1, caractérisé en ce que l'étape d'addition de la matière de charge (16) englobe:
le fait d'ajouter des particules réfractaires à la matrice (10).

7. Procédé de fabrication d'un recouvrement selon la revendication 1, caractérisé en ce que l'étape d'addition de la matière de charge (16) englobe:
le fait d'ajouter une matière dont le diamètre des particules est inférieur à un (1) millimètre.

8. Procédé de fabrication d'un recouvrement selon la revendication 1, caractérisé en ce que l'étape d'addition de la matière de charge (16) englobe:
le fait d'ajouter une matière dont le diamètre des particules est au moins égal à un (1) millimètre.

9. Procédé de fabrication d'un recouvrement selon la revendication 1, caractérisé en ce que l'étape d'addition de la matière de charge (16) englobe:
le fait d'ajouter de la poudre de PTFE conjointement avec des fibres de verre.

10. Procédé de fabrication d'un recouvrement selon la revendication 1, caractérisé en ce que l'étape d'addition de la matière de charge (16) englobe:
le fait d'ajouter de la poudre de PTFE conjointement avec des fibres céramiques.

11. Procédé de fabrication d'un recouvrement selon la revendication 1, caractérisé en ce que l'étape d'addition de la matière de charge (16) englobe:
le fait d'ajouter de la poudre de PTFE conjointement avec des fibres de quartz et avec des particules de feldspath.

12. Procédé de fabrication d'un recouvrement selon la revendication 1, caractérisé en ce que la matière de renforcement (22) est une matière tissée.

13. Procédé de fabrication d'un recouvrement selon la revendication 1, caractérisé en ce que la matière de renforcement (22) est une matière tricotée.

14. Procédé de fabrication d'un recouvrement selon la revendication 1, caractérisé en ce que la matière de renforcement (22) est une matière tressée.

15. Procédé de fabrication d'un recouvrement selon la revendication 1, caractérisé en ce que la matière de renforcement (22) est une matière non tissée.

16. Procédé de fabrication d'un recouvrement selon la revendication 1, caractérisé en ce qu'on effectue l'étape d'enroulement en spirale de la matière de renforcement (22) au cours de la réticulation de la matrice (10).
